

## UNITED STATES PATENT OFFICE

HANS REIHLLEN, OF KARLSRUHE, GERMANY, ASSIGNOR TO MILTON M. ADLER, OF NEWARK, NEW JERSEY

## PYROTECHNIC DEVICE

No Drawing.

Application filed March 19, 1927. Serial No. 176,833.

My invention relates to fireworks which are set in action by means of impact, or friction, or heat, and which show a flame action accompanied by a series of lively reports; such action taking place in such a way that the article does not explode in mass but rather divides itself into smaller particles which produce, in rapid succession, small, harmless explosions.

Up to date such fireworks were made with poisonous yellow phosphorus, potassium chlorate and organic binding materials, such as shellac or gum.

Fireworks made in accordance with my invention are entirely free from poisonous materials. According to the invention sulphur phosphorous compounds and particularly phosphorous sesquisulfide are used as the active agent. This I have found is a complete and harmless substitute for the poisonous phosphorus. To produce oxygen, there may be used potassium chlorate or potassium perchlorate and for practical purposes both of them. As a binder there are used magnesium chloride and magnesium oxide, a cementitious mixture generally known as "sorell cement". In order to produce the explosive mass, I proceed as follows:

Phosphorous sesquisulfide is introduced into a water mixture of potassium chlorate and potassium perchlorate to which has been added a cement mixture consisting of magnesium chloride and magnesium oxide. This mixture is then formed into discs or other shapes or spread on a suitable surface and dried.

The sulphur phosphorous compounds, as for instance phosphorous sesquisulfide, are best not used in finely powdered form. The ordinary phosphorous sesquisulfide should, therefore, be transformed into crystals of appropriate size by recrystallization with carbon bisulfide or other solvents. The coarser graining of the phosphorous sesquisulfide attained in this way makes for greater durability and a hardening of the composition of the mass or rather the discs made therefrom, as well as lessening the sensitivity to friction and danger from fire.

On the other hand, it has been found important to use the potassium perchlorate in the very finest powdered form, although the chlorate does not need to be so finely ground. The change of the perchlorate into the desired pulverized form can, for instance, be expediently produced by protracted tumbling in a pebble mill, with the addition of an effective auxiliary substance which facilitates the grinding, as for instance, fine sand.

As an example of the mixture, I dissolve 12 grams of crystallized magnesium chloride in 30 grams or more of water, and after adding 8 grams of potassium chlorate and then a mixture of 32 grams of potassium perchlorate and 8 grams of sand, I stir these ingredients into a thick paste. Into this mixture I incorporate 24 grams of burned magnesite ( $MgCO_3$ ) and then add 14 grams of phosphorous sesquisulfide, and mix very thoroughly. Out of this paste discs of the desired size are made and dried at moderate temperatures, as for instance, 40 to 70 centigrade. The discs may also be used, for instance, in the following way: that a number of them may be pasted next to each other on paper or paper strips. By igniting the paper, the individual discs or pellets can be made to explode one after the other, with a loud report. Also, in its wet state, the composition may, for instance, be deposited on a fuse and then dried. In burning the fuse, the desired harmless partial explosions follow each other in rapid succession.

In order to produce the oxygen, there may be used, in place of the potassium chlorate and potassium perchlorate, such other chlorates and perchlorates as e. g. of sodium, of magnesium, or of the alkaline earths. When such substitutes are used, it is desirable to cover the finished discs or other forms with suitable protective coatings, as for instance, those made of collodion.

Pyrotechnic articles made in accordance with the above invention have the advantage of being entirely free from poisonous substances. With this preparation the organic binding material and adhesives heretofore

considered indispensable, are now no longer necessary. In igniting the disc at one point, there is neither a complete burning up of the disc or an undesired explosion thereof; on the contrary, the flame dies out of its own accord regardless whether there is an accumulation of small discs or one larger one.

Claims.

- 10 1. Fireworks containing at least a sulphur phosphorous compound and containing chlorate to produce oxygen and using as a binding material, a sorell cement.
- 15 2. Fireworks containing phosphorous sesquisulfide, potassium chlorate, potassium perchlorate, sorell cement and sand.
- 20 3. A method of producing fireworks characterized in that phosphorous sesquisulfide in crystalline form is mixed with potassium chlorate and very finely pulverized potassium perchlorate, magnesium chloride and magnesium oxide, in connection with a liquid, and the mixture then dried.

In testimony that I claim the invention set forth above I have hereunto set my hand this 26th day of February, 1927.

HANS REIHLEN.

30

35

40

45

50

55

60

65